

# UNITED STATES PATENT OFFICE.

COLUMBUS D. STOVALL, OF LEXINGTON, KENTUCKY.

## ALLOY.

1,376,656.

Specification of Letters Patent.

Patented May 3, 1921.

No Drawing.

Application filed June 7, 1920. Serial No. 387,218.

To all whom it may concern:

Be it known that I, COLUMBUS D. STOVALL, a citizen of the United States, residing at Lexington, in the county of Fayette and State of Kentucky, have invented certain new and useful Improvements in Alloys, of which the following is a specification.

This invention relates to certain improvements in alloys and has relation more particularly to an alloy especially designed and adapted for use in connection with dentistry, and it is an object of the invention to provide a novel and improved alloy which is substantially non-oxidizable and which is hard, elastic and tenacious.

It is also an object of the invention to provide a novel and improved alloy which is of a good golden color, possessing the elasticity of tempered steel and which is high-fusing.

My improved alloy comprises the following ingredients mixed in substantially the proportions given:

|               |                  |         |
|---------------|------------------|---------|
| Plate (22 K.) | 72               | grains. |
| Nickel        | 13 $\frac{1}{2}$ | grains. |
| Copper        | 16 $\frac{1}{2}$ | grains. |
| Platinum      | 2                | grains. |

The nickel and copper, when combined with the remaining constituents, result in a finished product of a good golden color and an elastic, rigid, hard, high-fusing, tenacious metal, and in practice the fused mass is 30 preferably made into plates rolled to the desired thickness.

It has been fully established in practice that my improved alloy is substantially non-oxidizable and is particularly adapted for 35 use in connection with dentistry as the alloy will not discolor and is not affected by ordinary acids. It has also been fully established that annealing does not affect the elasticity or tenacity of my improved alloy. 40

I claim:

An alloy comprising gold, nickel, copper and platinum in the proportions described.

In testimony whereof I hereunto affix my signature.

COLUMBUS D. STOVALL.